

# United States Patent

[11] 3,622,378

[72] Inventor **Thomas J. Proffitt, Jr.**  
Kinston, N.C.  
[21] Appl. No. **751,345**  
[22] Filed **Aug. 9, 1968**  
[45] Patented **Nov. 23, 1971**  
[73] Assignee **E. I. du Pont de Nemours and Company**  
Wilmington, Del.

3,093,591 6/1963 Freese..... 252/8.8  
3,105,500 10/1963 Wilson et al..... 117/139.50  
3,277,079 10/1966 Press..... 117/139.50  
3,402,127 9/1968 Mowe..... 252/8.8

Primary Examiner—William D. Martin  
Assistant Examiner—J. E. Miller, Jr.  
Attorney—E. Leigh Hunt

[54] **FIBERS WITH ANIONIC-CATIONIC FINISH**  
1 Claim, No Drawings

[52] U.S. Cl. .... **117/138.8 N,**  
8/115.6, 117/138.8 U, 117/138.8 F, 117/139.5  
CQ, 252/8.75, 252/8.8  
[51] Int. Cl. .... **C09k 3/16,**  
D06m 3/16, D06m 3/30  
[50] Field of Search. .... **117/139.50,**  
138.8 U, 138.8 N, 138.8 F; 8/115.6; 252/8.75, 8.8  
[56] References Cited  
UNITED STATES PATENTS

3,003,954 10/1961 Brown ..... 252/8.8

**ABSTRACT:** A textile fiber having a finish coating of compatibilized cationic and anionic components comprising from 0.06 percent to about 3 percent by weight of the fiber, said coating comprising a mixture of (a) an organic anionic surfactant containing at least one alkyl or alkenyl group having from eight to 20 carbon atoms; (b) an organic cationic nitrogen containing surfactant having at least one long chain alkyl or alkenyl group of eight to about 20 carbon atoms; and (c) a compatibilizing quantity of an organic amphoteric nitrogen containing surfactant having at least one alkyl or alkenyl group of eight to 20 carbon atoms.

## FIBERS WITH ANIONIC-CATIONIC FINISH

## BACKGROUND OF THE INVENTION

5

## 1. Field of the Invention

This invention concerns surfactants for textile fibers and, more specifically, organic fiber-finishing compositions containing both cationic and anionic components.

## 2. Description of the Prior Art

In the production of textile fibers, it is customary to apply to the surfaces thereof compositions such as oils or antistats to protect the fiber from damage by contact with machinery and for other reasons such as to give the fiber antistatic properties and to improve its tactile aesthetics. In the trade these compositions are customarily called "finishes" and are made up of various chemical compounds depending upon their anticipated function. It is frequently desirable to use either cationic or anionic organic surfactants as fiber finishes, each carrying particular properties to dispose the fibers in a desirable manner. The desirability of a water-soluble finish containing both anionic and cationic compounds, for instance, a good anionic antistat and a good cationic softener, is recognized in the trade. However, such a finish composition is not known because of the incompatibility of the two types of ingredients. Upon mixing of the anionic and cationic agents, precipitation and sludge-like formation invariably occurs. Thus, the two agents are called "incompatible." Even when one of the agents is deposited on the fibers and at a later stage in processing the other agent is applied, undesirable solid deposits form and, more than likely, the finished yarn has neither of the desirable properties that each agent was designed to produce.

## SUMMARY OF THE INVENTION

The invention in its broad scope is defined as a textile fiber containing on its surface from 0.06 percent to 3 percent by weight of a finish comprising an organic anionic, an organic cationic, and an organic amphoteric surfactant, the amount of amphoteric being at least 3 percent of the total solids weight of the finish composition.

The invention in its narrower aspect is defined as a textile fiber having a finish coating of compatibilized cationic and anionic components comprising from 0.06 percent to about 3 percent by weight of the fiber, said coating comprising a mixture of (a) an organic anionic surfactant containing at least one alkyl or alkenyl group having from eight to 20 carbon atoms; (b) an organic cationic nitrogen containing surfactant having at least one long chain alkyl or alkenyl group of eight to about 20 carbon atoms; and (c) a compatibilizing quantity of an organic amphoteric nitrogen containing surfactant having at least one alkyl or alkenyl group of eight to 20 carbon atoms.

## DESCRIPTION OF THE PREFERRED EMBODIMENTS

It has been unexpectedly found that organic anionic surfactants and organic cationic surfactants are compatibilized in a textile fiber finish by inclusion in the finish bath of at least 3 percent, based on the combined solids weight of the anionic and cationic ingredients, of an organic amphoteric compound. The inclusion of the amphoteric precludes precipitation and sludge formation in the composite finish.

The term organic cationic surfactant refers to a salt that dissociates in solution into an organic cationic surfactant. The organic cationic surfactants included in the chemical combination of this invention are organic nitrogen compounds having at least one long chain alkyl or alkenyl group of eight to about 20 carbon atoms. The most preferred cationic surfactants con-

tain a quaternary nitrogen atom. Typical organic cationic salts useful as surfactants in the practice of this invention comprise:

2

TABLE I.—CATIONIC SURFACTANTS

| 10 | Name                                            | Structure                                                                                    |
|----|-------------------------------------------------|----------------------------------------------------------------------------------------------|
| 15 | a. N-cetyl-N-ethyl-morpholinium-ethyl sulfate.  |                                                                                              |
| 20 | b. Cocotrimethylammonium chloride.              |                                                                                              |
| 25 | c. Cocomethyldi(hydroxyethyl)ammonium chloride. | Same as (b) except replace two methyl groups with hydroxyethyl groups.                       |
| 30 | d. Distearyldimethylammonium chloride.          | Same as (b) except replace the coco substituent and one CH3 substituent with stearyl groups. |

Organic anionic surfactant refers to a salt that dissociates in solution into an organic anionic surfactant. The organic anionic surfactants included in the chemical composition of this invention contain at least one alkyl or alkenyl group having from eight to 20 carbon atoms. The most preferred are the potassium and sodium salts of the compound having a phosphate or a sulfate group. Typical organic anionic salts useful as surfactants in the practice of the present invention comprise:

TABLE II.—ANIONIC SURFACTANTS

| 50 | Name                                       | Structure                                                            |
|----|--------------------------------------------|----------------------------------------------------------------------|
| 55 | a. Potassium mono- and ditooctylphosphate. |                                                                      |
| 60 | b. Sodium laurylsulfate.                   | Lauryl-O-S-O3Na. where X=1 or 2.                                     |
| 65 | c. Potassium mono- and didecylphosphate.   | Same as (a) except substitute a decyl group for the iso-octyl group. |
| 70 | d. Sodium-N-cyclohexyl-N-palmitoyltaurate. |                                                                      |

An organic amphoteric surfactant refers to an organic surfactant having both acid and basic properties. The amphoteric surfactants useful in the practice of the present invention are defined as nitrogen-containing organic compounds having at least one alkyl or alkenyl group of eight to 20 carbon atoms. The most preferred contain a carboxyl group or the sodium salt of a carboxyl group. Typical amphoteric surfactants useful in the practice of this invention comprise:

TABLE III.—AMPHOTERIC SURFACTANTS

The new finish combination is preferably made up in batch form and then applied to the textile fiber. However, the new combination may be applied to the fiber in stepwise fashion; for example, the anionic agent may be applied to the fiber at one point in the process and, at a later point, the cationic and amphoteric compounds may be applied. In the former process, it is preferable to avoid mixing the anionic and cationic ingredients before the amphoteric is admixed. In many cases, however, the amphoteric destroys the precipitate formed on mixing of the anionic and cationic ingredients.

formed on mixing of the anionic and cationic ingredients. An advantage of the new finish is that it is water-dispersible. This advantage is noteworthy in that water is inexpensive and readily available and easy to clean from machine parts, etc. Preferably, the amphoteric compound is added to a vessel containing the required volume of water. Then, the anionic and cationic ingredients are admixed. Usually, concentrations of from 1 to 20 percent solids of the new finish combination in water are applied to running fibers by means of a finish applicator. Applications to produce a solids content of finish ingredients on the finished yarn of from 0.06 percent to 3 percent based on the total weight of the finished yarn are satisfactory.

The new finish combination or any ingredient thereof may be applied to textile fibers at any place in the production process. Thus, the combination or any part thereof can be an-

plied as a predraw application or postdraw application or even as an overlay finish.

The invention includes any known textile fiber and is particularly advantageous with fibers based on polymers and copolymers of polyethylene terephthalate, nylon, and polyacrylonitrile. These fibers have a high volume in the apparel markets where adequate finishing techniques are demanded to prevent the fiber from irritating the skin or from being excessively electrostatic.

The invention will be further illustrated by the following examples which illustrate the invention but are not intended to be delimitative.

### EXAMPLES I-XIII

65 These examples show the amount of amphoteric compound necessary to compatibilize the anionic and cationic surfactants shown in the above tables in all proportions.

To a beaker containing a volume of water is added an amphoteric surfactant selected from table III, an anionic surfactant selected from table II and a cationic surfactant selected from table I. The amount of amphoteric necessary to compatibilize the cationic to anionic is recorded. Results are as follows:

| Example | Cationic surfactant from Table I | Anionic surfactant from Table II | Amphoteric surfactant from Table III | Finish solution concentration (percent solids in water) | Minimum percent by weight <sup>1</sup> of amphoteric to compatibilize |
|---------|----------------------------------|----------------------------------|--------------------------------------|---------------------------------------------------------|-----------------------------------------------------------------------|
| I       | a                                | a                                | a                                    | 10                                                      | 10                                                                    |
| II      | b                                | a                                | a                                    | 10                                                      | 12                                                                    |
| III     | b                                | a                                | b                                    | 10                                                      | 13                                                                    |
| IV      | c                                | a                                | a                                    | 10                                                      | 15                                                                    |
| V       | d                                | a                                | b                                    | 5                                                       | 22                                                                    |
| VI      | d                                | a                                | c                                    | 5                                                       | 25                                                                    |
| VII     | b                                | b                                | d                                    | 5                                                       | 25                                                                    |
| VIII    | b                                | b                                | e                                    | 5                                                       | 25                                                                    |
| IX      | d                                | a                                | f                                    | 5                                                       | 33                                                                    |
| X       | d                                | b                                | e                                    | 5                                                       | 35                                                                    |
| XI      | d                                | b                                | d                                    | 5                                                       | 55                                                                    |
| XII     | d                                | d                                | a                                    | 10                                                      | 60                                                                    |
| XIII    | d                                | b                                | g                                    | 5                                                       | 95                                                                    |

<sup>1</sup> (Amphoteric solids weight + finish solids weight)  $\times 100$ .

Each of the above finish compositions is satisfactory as a textile fiber finish. When each of the cationic surfactants is mixed with the anionic surfactants without the addition of amphoteric compound, undesirable precipitation invariably occurs.

#### EXAMPLES XIV-XVII

These examples show the application of the finish combinations to textile fibers and show improvement in static electricity properties of the fibers resulting thereby.

The static electricity measurements are determined as follows: A Beckman Micro-microammeter Model-5 manufactured by Beckman Instruments Inc., Fullerton, Calif. with a DC potential of 210 volts and a resistance of 1 megohm is set up. A thin plate of electrically resistant material having four metal prongs mounted perpendicularly at each corner of a 1.25 inch square (3.2 cm. square) thereon is fabricated and connected to the Micro-microammeter in such a way that upon connecting two pairs of prongs (one pair to negative and one pair to positive 210 volts) current will flow in the system when a sample is on the prongs. The yarn to be tested for static electricity is wound on a 3-in. (7.6 cm.) long 2-in. (5.1 cm.) diameter core to a thickness of about  $\frac{1}{4}$ -in. (0.64 cm.). The core containing the yarn is placed lengthwise against the four prongs of the electrical system, and the amount of current flowing through the circuit is measured. Knowing the potential and the amount of current, the resistance is calculated and its logarithm is recorded.

The finish compositions are metered onto the yarn from aqueous solution by means of a metering pipette.

Yarns used for these examples are as follows:

I. 70-denier/34-filament polyhexamethyleneadipamide (nylon) having 2 "Z" turns per inch (0.79 turns/cm.) twist and containing 0.3 percent by weight  $TiO_2$ . When finished the finish level on this yarn is 0.5 percent solids finish ingredients based on the weight of the finished yarn.

II. 70-denier/34-filament polyethylene terephthalate having essentially no twist and containing 0.3 percent  $TiO_2$ . In example XVI the yarn is finished to a level of 0.2 percent solids finish ingredients based on the weight of the finished yarn.

III. 75-denier/30-filament yarn comprising a copolymer of 94 percent acrylonitrile and 6 percent methyl acrylate having 0.3 "Z" turns per inch (0.12 turns/cm.) twist and 0.4 percent  $TiO_2$ . In examples XVII the yarn is finished to a level of 0.2 percent by weight solids finish ingredients based on the weight of the finished yarn.

#### EXAMPLE XIV

The finish-free nylon yarn is coated with a 10 percent by weight, aqueous solution comprising 20 parts by weight of the amphoteric of table III-a, 40 parts by weight of the anionic of table II-a, and 40 parts by weight of the cationic of table I-b. The finish level is 0.5 percent by weight solids finish based on the weight of the finished yarn. Log R of the finished yarn is 7.5 at 65 percent relative humidity.

A comparable nylon yarn containing no finish gives a Log R value at the same humidity of approximately 16.5 indicating a degree of static electricity unfavorable for a textile fiber.

#### EXAMPLE XV

The same nylon starting material as used for example XIV is 20 covered with a 10 percent aqueous finish composition comprising 10 parts by weight of the amphoteric surfactant of table III-a, 10 parts by weight of the cationic surfactant of table I-a and 80 parts by weight of the anionic surfactant of table II-a. The yarn is finished to a level of 0.5 percent by 25 weight solids finish based on the weight of the finished yarn. Log R at 65 percent relative humidity is 7.5.

#### EXAMPLE XVI

30 The polyethylene terephthalate yarn is coated with a 20 percent by weight aqueous solution comprising the complex anionic surfactant formed by combining 11.6 parts by weight of mono- and didecyl-phosphoric acids (50 percent mono 50 percent di) with 8.4 parts of triethanolamine, 40 parts by weight of a nonionic surfactant of a 12- to 18-carbon synthetic 35 primary alcohol condensed with polyoxyethylene so that the weight of polyoxyethylene is 60 percent of the total weight of the molecule, and 20 parts of the amphoteric of table III-d, and 20 parts by weight of the cationic surfactant of table I-b. 40 Log R value of the finished yarn is 7.5 as compared to a Log R value of 17.2 for an identical yarn containing no finish on its surface.

#### EXAMPLE XVII

45 The yarn of acrylonitrile and methylacrylate is coated with a 20 percent by weight aqueous solution comprising 10 parts by weight of a cationic surfactant consisting of dicocodimethylammonium chloride, 30 parts by weight of the amphoteric of table III-a, 10 parts by weight of the anionic 50 surfactant used in example XVI and 50 parts by weight of the nonionic surfactant used in example XVI. The yarn is finished to a level of 0.2 percent by weight solids finish based on the total weight of the finished yarn. The Log R value is 11.8 at 20 percent relative humidity as compared to a Log R value of 16.9 for an identical yarn having no finish on its surface.

#### EXAMPLE XVIII

This example shows the combination, in a single bath, of cationic and anionic surfactants in a composition containing other ingredients, by use of an amphoteric surfactant.

To a vessel containing a volume of water is added 3 parts, by weight, of the amphoteric of table III-a, 27.7 parts, by weight, of a cationic surfactant comprising the reaction product of stearic acid and diethanolamine quaternized with dimethylsulfate; and 69.3 parts of a mixture comprising 16.6 parts of an anionic surfactant comprising sulfated peanut oil partially neutralized with sodium hydroxide, 8.2 parts by weight of oleic acid, 1.4 parts of 45 percent aqueous solution of potassium hydroxide, 3.1 parts of triethanolamine (the reaction product of the latter three ingredients is anionic), 1.4 parts by weight of diethylene glycol (nonionic), 35.5 parts, by weight, of number-50 mineral oil, 3.1 parts, by weight, of the anionic surfactant comprising o-phenylphenol sodium salt. The solution comprises 17 percent, by weight, nonaqueous ingredients. The resulting surfactant mixture is entirely suitable for textile fibers. When an identical mixture is made without the

amphoteric ingredient, a lumpy consistency develops.

The finish is used as a predraw finish on nylon yarn, and the yarn is found to have excellent antistatic and frictional properties.

The present invention teaches how to compatibilize anionic and cationic surfactants in textile fiber finish compositions. In so doing, new paths are opened to experiment with new anionic, cationic, and amphoteric surfactants for fibers. It has now been found possible to use certain surfactants having outstanding properties in systems which until now were considered impractical.

What is claimed is:

1. In a process for coating textile fibers with surfactant composition to impart improved frictional and antistatic proper-

ties, wherein said composition consists essentially of (a) an organic anionic surfactant having an alkyl or alkenyl group of eight to 20 carbon atoms and (b) an organic cationic nitrogen-containing surfactant having a long-chain alkyl or alkenyl group of eight to 20 carbon atoms, and the proportion of said surfactants is such that surfactants (a) and (b) tend to precipitate out of the composition; the improvement which comprises including in the composition an organic amphoteric nitrogen-containing surfactant having an alkyl or alkenyl group of eight to 20 carbon atoms, the amount of amphoteric surfactant being sufficient to prevent surfactants (a) and (b) from precipitating.

15

\* \* \* \* \*

20

25

30

35

40

45

50

55

60

65

70

75